

## UNITED STATES PATENT OFFICE

ROBERT E. WILSON, OF CHICAGO, ILLINOIS, ASSIGNOR TO STANDARD OIL COMPANY, OF WHITING, INDIANA, A CORPORATION OF INDIANA

## PREDILUTED LUBRICATING OIL

No Drawing.

Application filed July 2, 1928. Serial No. 290,051.

This invention relates to prediluted lubricating oils which are intended to be in a condition of substantial equilibrium with respect to dilution under average operating conditions of automobile or other motors, and which do not, therefore, materially change in viscosity during normal use. The invention relates particularly to such oils comprising low pour test lubricants derived from wax-bearing crude.

In accordance with the present invention wax-bearing lubricating oil, for example a residual oil derived from the reduction of once pressed wax distillate, is diluted with heavy naphtha which is suitable for use as an equilibrium diluent. The diluted oil is chilled and pressed, settled or centrifuged to remove wax. The dewaxed oil is embodied in a prediluted lubricating oil, the heavy naphtha constituting the diluent or a part of the diluent, thereof. If, in any case, it is necessary to employ, for wax removal, a larger amount of naphtha than is appropriate in the finished lubricant, the excess may be readily removed by evaporation at any time after dewaxing. In such a case, it is preferred to employ a slightly lighter naphtha and to remove the lighter portion after dewaxing, so that naphtha of the appropriate composition and in proper amount remains in the oil.

The invention will readily be understood from the following description of a specific example.

A satisfactory prediluted medium motor oil may be constituted as follows:

|                                                                   | Per cent |
|-------------------------------------------------------------------|----------|
| Pressed paraffin base oil (viscosity 300 sec. Saybolt at 100° F.) | 36       |
| Filtered cylinder stock                                           | 18       |
| Low cold test naphthenic base oil                                 | 36       |
| Heavy naphtha (300 to 460° F. boiling range)                      | 10       |

The pressed paraffin base oil is prepared as follows. Wax distillate, also known as paraffin distillate, is pressed once in the usual way for removal of wax. Thereafter the distillate is reduced for the production of light lubricating oils and a red oil of about 300 sec. Saybolt viscosity at 100° F. The average yield of such a heavy red oil is about 15%.

To 36 parts of this red oil 10 parts of heavy naphtha of the boiling point range 300 to 460° F. are added, giving a mixture with a viscosity of about 80 sec. at 100° F. This mixture is chilled in the usual manner to about -10° F. and the wax is removed by pressing or centrifuging. The low cold test oil thus obtained may be blended directly with the cylinder stock and naphthenic base oil to give a diluted lubricating oil of the composition set forth above.

Although the present invention has been described in connection with details of a specific example, it must be understood that such details are not intended to be limitative upon the scope of the invention except in so far as included in the accompanying claims.

I claim:

1. The method of producing a prediluted lubricating oil which consists in adding heavy naphtha to a wax-bearing lubricating oil, chilling the diluted oil, removing wax therefrom and embodying the dewaxed oil and heavy naphtha in a prediluted lubricating oil.

2. The method of producing a prediluted lubricating oil which consists in adding heavy naphtha to wax-bearing lubricating oil in sufficient quantity to facilitate wax removal at low temperatures, chilling the mixture, removing wax therefrom and mixing the oil with other lubricant oils.

3. The method of producing a prediluted lubricating oil which consists in pressing paraffin distillate, reducing said distillate thereby by producing a heavy lubricating oil, diluting said heavy oil with heavy naphtha, chilling the mixture and removing wax therefrom, and blending the mixture with other lubricant oils.

4. The method of producing a prediluted lubricating oil which consists in pressing paraffin distillate, reducing said distillate thereby by producing a heavy lubricating oil, diluting said heavy oil with heavy naphtha, chilling the mixture and removing wax therefrom, and blending the mixture with a naphthenic base lubricating oil.

5. The method of producing a prediluted lubricating oil which consists in pressing paraffin distillate, reducing said distillate there-

by producing a heavy red oil, diluting said heavy red oil with heavy naphtha, chilling the mixture and removing wax therefrom, and blending the mixture with low cold test naphthenic base lubricating oil and filtered cylinder stock.

6. The method of preparing a prediluted motor lubricating oil which consists in pressing a wax distillate, reducing said distillate to a 15% bottom having a viscosity of about 10 300 sec. Saybolt at 100° F., adding heavy naphtha having a boiling range between about 300 and 460° F., to said residual oil in the proportion of about 10 parts of naphtha to about 36 parts of the red oil, thereby giving a mixture with a viscosity of about 80 sec. Saybolt at 100° F., chilling the mixture to about -10° F., removing wax and blending the dewaxed mixture with about 18 parts 15 of filtered cylinder stock and about 36 parts 20 of low cold test naphthenic base lubricating oil.

In testimony whereof I have hereunto set my hand this 31st day of May, 1928.

25 ROBERT E. WILSON.

30

35

40

45

50

55

60